

## UNITED STATES PATENT OFFICE.

MAX BIELEFELDT, OF BERLIN, GERMANY.

## BLASTING COMPOSITION.

SPECIFICATION forming part of Letters Patent No. 789,252, dated May 9, 1905.

Application filed January 6, 1902. Serial No. 88,607.

*To all whom it may concern:*

Be it known that I, MAX BIELEFELDT, a subject of the German Emperor, residing at Berlin, Germany, have invented certain new and useful Improvements in Blasting Compositions, of which the following is a specification.

Many attempts have been made to modify the composition of dynamite by means of suitable admixtures, so as to render it safe for use in "fiery" coal-mines without materially reducing its disruptive power. For instance, the blasting composition known as "fire-damp" dynamite ("wetter" dynamite) contains 38.5 per cent. of rye-flour and one per cent. of wood-flour, which additions, however, considerably reduce the disruptive power of the dynamite. In order to avoid this defect, I substitute for about half the quantity of cereal flour and cellulose-flour hydrocarbons which have a high molecular weight and are rich in carbon, such as liquid paraffin, ceresin, naphthalene, and anthracene. Dynamites containing approximately from thirty-five to forty-five per cent. of nitroglycerin thereby acquire a considerably higher disruptive power in comparison with the products containing the full quantity of the said flours. The power of these explosives may be further enhanced by adding a suitable quantity of ammonium nitrate, and a small part of the latter may be replaced by potassium or sodium nitrate.

An eminently safe and powerful dynamite may be obtained by mixing nitroglycerin with hydrocarbons of high molecular weight, flour of cereals and cellulose, and inorganic nitrates, preferably ammonium nitrate, in such proportions that the finished explosive composition contains about thirty-five to forty-five per cent. of nitro compounds and that the quantity of hydrocarbons of high molecular

weight is from one-fourth to one-half that of the organic nitro compound and is approximately equal to the quantity of cereal and cellulose flour.

The following composition has been found to possess great disruptive power without being liable to cause explosions of fire-damp: forty parts of nitroglycerin, two parts of collodion-cotton, eight parts of paraffin-oil, (paraffinum liquidum,) four parts of naphthalene, twelve parts of rye-flour, two parts of wood-flour, twenty-seven parts of ammonium nitrate, (ammonia saltpeter,) five parts of potassium nitrate, (potash saltpeter.)

The principal object of the collodion-cotton in the above example is to gelatinize the blasting composition. If this effect is not desired, the collodion-cotton may be omitted.

What I claim is—

1. A blasting composition containing nitroglycerin, a hydrocarbon of high molecular weight and rich in carbon, cereal flour, cellulose-flour and an inorganic nitrate, the quantity of the hydrocarbon being approximately from one-fourth to one-half the quantity of the organic nitro compound and approximately equal to the quantity of flour of cereals and cellulose, substantially as described.

2. A blasting composition composed of forty parts of nitroglycerin, two parts of collodion-cotton, eight parts of paraffin-oil, four parts of naphthalene, twelve parts of rye-flour, two parts of wood-flour, twenty-seven parts of ammonium nitrate, five parts of potassium nitrate, substantially as described.

In testimony whereof I have hereunto set my hand in presence of two subscribing witnesses.

MAX BIELEFELDT.

Witnesses:

LUDWIG MOELLER,  
A. KREFT.